

Feb. 11, 1930.

V. BENDIX

1,746,925

BRAKE DRUM

Original Filed May 2, 1928



Inventor

VINCENT BENDIX

By

Mr. W. McConkey

Attorney

## UNITED STATES PATENT OFFICE

VINCENT BENDIX, OF SOUTH BEND, INDIANA, ASSIGNOR TO BENDIX BRAKE COMPANY,  
OF SOUTH BEND, INDIANA, A CORPORATION OF ILLINOIS

## BRAKE DRUM

Original application filed May 2, 1928, Serial No. 274,677. Divided and this application filed February 28, 1929. Serial No. 343,319.

This invention relates to improvements in brake drums and is a division of my application Serial No. 274,677, filed May 2, 1928, patented July 16, 1929 No. 1,720,815.

5 In the past brake drums have been made of relatively easily corrodible material such as iron. As this ferruginous base metal corrodes, not only does it become unsightly, but it also becomes seriously weakened by reason 10 of the fact that the iron of relatively high tensile strength is replaced by a deposit of iron oxide which possesses substantially no strength. This corrosion or oxidation is accelerated during use because of the fact that 15 the temperature of the drum is raised by the generated frictional heats. Upon continued use of the brake drum, it is found that it tends to distort and lose its initial circular shape. This materially lowers the braking efficiency.

20 The corrosion of the drum lowers the strength and hence accentuates this distortion.

It is an object of this invention to provide a structural material particularly well adapted to the manufacture of brake drums which 25 are of low corrodibility and of the desirable high tensile strength.

Another object is to provide a brake drum of high strength, low corrodibility and hardness.

30 Another object is to provide a novel composite brake structure of a ferruginous material and another metal.

A further object is to provide a brake drum of a ferruginous base metal with which is 35 combined certain other metals which increase the strength and lower the corrosion.

The single figure on the drawing is an enlarged and diagrammatic illustration of a 40 brake drum produced according to the invention.

As pointed out in my parent application, the availability, ease of manufacture and machining, and the relative cheapness of deep-draw steel recommends its use in brake drum 45 structures. Ordinary steel, however, is relatively easily corroded. When used in brake drums it is subjected to constant wettings and corrosion sets in. This, as is known, consists in oxidation of the iron and, as has been 50 pointed out, is accelerated by the frictional

heats. This corrosion is practically cumulative; the iron oxide which is formed not only does not provide a protective coating but accelerates subsequent corrosion or oxidation of the underlying body.

55 This disadvantage may in a measure be cured by manufacturing a drum from chromium, vanadium, zirconium or other alloy steels. These materials not only are characterized by extremely low corrodibility but are also of a high tensile strength. While these materials do present major advantages, they are considerably more expensive than the ordinary steel employed.

60 According to the purpose of this invention, a brake drum may be produced which presents all of the advantages of the alloy steels, and in addition provides certain added advantages.

65 In the application referred to there was described and claimed a brake drum which comprised a ferruginous foundation metal on the exterior of which was deposited a plating of chromium. The advantage of a thin coat of chromium or similar relatively non-oxidizable metals may be combined with the highly protective features of a thick coating of such metal. The present preferred method 70 of accomplishing these will serve to indicate the underlying principles of the invention. These advantages may be achieved by treating a brake drum, or the material from which 75 a brake drum is made, with metallic zinc so as to form a coating of zinc over the outer or exposed surface of the drum. It will be understood, of course, that if desired, the interior surface of the drum may similarly be treated or the treatment localized to any desired area.

80 As shown in the drawing, the zinc may be 85 cemented to the iron by galvanizing or sherardizing in the well known manner.

90 In the electro-chemical series zinc is given as electro-positive to iron. This is tantamount to saying that it has a greater solution pressure or tendency to dissolve. Therefore, when it is in contact with moisture, the zinc becomes the dissolving electrode and the iron the electrode on which the deposits are 95 formed. As a result, the zinc not only me- 100

chanically protects the iron, that is to say forms a protective coating thereover, but it also provides electro-chemical protection.

The sherardizing or metallic cementation 5 may be carried out according to any accepted practice. These methods in general consist in cleaning the metal to be treated and then packing it in zinc dust within an air-tight metal container. The container is then heated and tumbled. As a general rule "blue dust" or a mixture of "blue dust" and zinc oxide are employed. These processes are generally carried out at temperatures ranging from 350° to 375° C., the temperature 10 employed being dependent upon the desired zinc content of the alloy and the composition of the zinc dust. For the present use it is preferable that the treatment be continued for a sufficient period of time so as to insure a 15 substantial quantity of zinc in the outer coating after diffusion has taken place.

The resulting structure then comprises a metallic member made up of iron and a zinc iron alloy, the outer surface of the member 25 having a larger percentage of zinc. During continued use, particularly at high temperatures, the zinc tends to diffuse through the iron and decreases the concentration of zinc in the outer layer. Since the zinc iron alloy, 30 like the zinc, is anodic to iron, it is necessary only to carry out the process sufficiently long to insure a zinc content which will adequately protect the iron.

After the ferruginous material has been 35 treated with zinc so as to form a coating or skin of a zinc compound, the surface may then be plated with the desired metal of low 40 corrodibility, in the present instance with chromium. This may be carried out by the electrodeposition method, explained in the copending application above referred to.

As the result of the provision of an intermediate layer of zinc, the deposited skin or film of chromium may be very thin and hence no great care need be exercised to avoid perforations. If such perforations do occur they will have no deleterious effect since, as has been pointed out, the zinc provides electro-chemical protection for the iron. If the 50 moisture has access to the zinc coating, this will slightly tarnish, but its unsightliness is in no way comparable to that of iron oxide.

The metal zinc has been described as merely 55 indicative of a number of specific metals which may be used. As has been explained, the protective feature of zinc depends in part on its electro-chemical characteristics; thus in place of zinc the iron may be coated with any suitable substance which is electro- 60 positive to it and upon which may be formed an adherent coat of the plating metal. Similarly in lieu of chromium, one may employ other metals such as nickel and cadmium, which are depositable as lustrous and non-oxidizing films.

While I have described the preferred embodiment of my invention, it is to be understood that this is given by way of example, for since the underlying principles may be incorporated in other specific structures I do not intend to be limited to that described except as such limitations are clearly imposed by the appended claims.

I claim:

1. A brake drum comprising a ferruginous material having an exterior surface of chromium and an intermediate layer of zinc.

2. A brake drum comprising a ferruginous foundation metal on which is superimposed a plurality of layers of metals of different 70 80 corrosion characteristics.

3. A brake drum of ferruginous metal having an outer coating of a lustrous and relatively non-corrodible metal, and an interposed portion of a metal which provides electro-chemical protection for the ferruginous metal.

4. A brake drum comprising a ferruginous foundation metal having an exterior surface of a metallic substance of low corrodibility 90 and a second metallic substance interposed between the said surface and foundation metal which is anodic to the ferruginous metal.

5. A brake drum comprising a foundation metal, an exterior surface comprising a metallic substance of lower corrodibility than the foundation metal and an intermediate portion having embodied therein a metallic substance which is anodic to the foundation metal.

6. A brake drum comprising a foundation metal having an exterior surface of chromium and an intermediate portion in which zinc is embodied.

7. A brake drum comprising a ferruginous foundation material, the interior frictional engaging surface of which is surfaced with chromium.

8. A brake drum comprising a ferruginous foundation metal having an interior frictional engaging surface of lower corrodibility than the foundation metal.

9. A brake drum comprising a ferruginous foundation metal having an interior frictional engaging surface which contains chromium.

10. A brake drum comprising a ferruginous foundation metal with which two other metals of differential physical characteristics are associated.

11. A material adapted for use in the manufacture of brake drums comprising a ferruginous foundation metal having a zinc containing portion and a chromium containing portion overlying the zinc containing layer.

12. A brake drum comprising a ferruginous core, a zinc containing layer on each face of the core and a relatively non-oxidiz-

able metal plated on the zinc containing layers.

13. A brake drum comprising a ferruginous foundation metal having layers of integrally bonded non-ferrous metals.

14. A brake drum comprising a ferruginous foundation metal having a galvanized portion and a relatively non-oxidizable metal plated on said portion.

15. A brake drum comprising a ferruginous foundation metal having a galvanized portion and a surface of chromium plated on said portion.

In testimony whereof I affix my signature.

VINCENT BENDIX.

5

10

25

30

35

40

45

50

55